

Patented Dec. 19, 1950

2,534,828

UNITED STATES PATENT OFFICE

2,534,828

ASPHALT BITUMINOUS BONDING COMPOSITION AND PROCESS OF PREPARATION

Lloyd J. Mitchell, Berkeley, and Harry J. Sommer, Lafayette, Calif., assignors to Shell Development Company, San Francisco, Calif., a corporation of Delaware

No Drawing. Application August 14, 1948,  
Serial No. 44,404

6 Claims. (Cl. 106—273)

1

This invention relates to improvements in bituminous compositions such as asphalt, asphalt cut-back and asphalt emulsions. More particularly, it is concerned with improving the bonding characteristics of such substances and with a method for carrying out the improvement.

It has been determined by numerous investigators that bituminous substances such as asphalt do not normally adhere to surfaces such as mineral aggregates, metals and other objects in the presence of water. It has been established that water will more or less readily displace asphalt films therefrom. The use of various additives to overcome this adverse characteristic has been widely recognized. Three main types of additives have been employed for this purpose. These include high molecular weight acids, soaps and amines. Various combinations of these have been used, and water-soluble materials such as metallic salts, have been used for priming the surface before coating with a bituminous material.

The configuration and characteristics of these additives vary widely, as would be expected. Some are applicable to basic rocks, such as limestone; others to acid rocks, such as granite, while certain species may be employed on any type of surface or with asphalts from a variety of sources.

One of the shortcomings to which most of these "adhesion agents" are subject is the tendency for the effect of the agent to decrease if the asphalt in which it is contained is subjected to aging or heating. This is a serious shortcoming from a practical standpoint, since it is advantageous to add the agent to the asphalt, cut-backs and road oils prior to shipment to road-laying or building sites. During such shipments, the asphalt, cut-backs and road oils are maintained for extensive periods at elevated temperature. This period of heating may continue for as long as a week or more; hence, any additive employed under such conditions should possess the ability to maintain its adhesion improving quality under these conditions.

Many amines are satisfactory for improving the adhesion characteristics of bituminous compositions as long as stability to heating is not a factor. However, it has been found that long-chain amines, such as octadecylamine, are unstable under heating conditions such as those described above. Likewise, cyclic amines, such as heptadecylimidazoline, are unstable under such conditions.

It is an object of the present invention to provide bituminous compositions having improved bonding characteristics. It is another object of this invention to provide a process for the preparation of such compositions. Other objects will become apparent during the following discussion.

2

Now, in accordance with the present invention, it has been found that oleophilic pyrimidines having a particular configuration possess a unique property which makes their use as anti-stripping agents in bituminous substances unexpectedly advantageous. It has been discovered that the adhesion effect of certain substituted pyrimidines in asphalt actually improves when the asphalt composition containing them is heated.

Still in accordance with this invention, it has been found that because of this unaccountable phenomenon, asphalt compositions containing the class of substituted pyrimidines described hereinafter are superior to asphalts containing the various amine-type adhesion agents, since the latter become poorer in adhesion characteristics when heat treated.

Bituminous substances which may be improved according to the present invention include especially pyrogerous residues, such as asphalts and pitches, as well as natural asphalts and tars, such as coal tar. Asphalts employed for the preparation of roads, airports and similar surfaces are especially suitable for the treatment to be described.

The substituted pyrimidines have the general structure:



Wherein each R is a hydrogen atom or an alkyl group and at least one R is an alkyl group having at least 10 carbon atoms.

Preferably, R<sub>1</sub> is the long-chain alkyl group having at least 10 carbon atoms. Typical groups include the decyl, dodecyl, tetradecyl, cetyl, ceryl and carnaubyl radicals. Another preferred structure includes those species wherein R<sub>2</sub>, R<sub>3</sub> and R<sub>4</sub> are short-chain alkyl radicals having 1-5 carbon atoms. These include both straight-chain and branched-chain radicals, such as methyl, ethyl, amyl, etc. The species which is especially preferred is 2 - heptadecyl - 4,6,6-trimethyl-3,4,5,6-tetrahydropyrimidine.

Substituted pyrimidines having the above preferred configuration may be prepared by processes already known. An especially suitable process comprises the reaction of a long-chain fatty acid with a 1,3-diamine.

Equimolecular quantities of the long-chain fatty acid and the substituted 1,3-diamine are heated in a suitable solvent (e. g., xylene) in the presence of an acid catalyst, with the azeotropic removal of water as it is formed. As the reaction proceeds and the rate of water formation decreases, the solvent is removed, and the kettle

temperature increased to 175°-200° C. When the theoretical amount of water has been collected, the reaction mixture is neutralized with calcium carbonate, and the product recovered by distillation. An actual working example is the reaction of stearic acid with 2-methyl-2,4-pentanediamine:

A solution consisting of one mole of stearic acid, one mole of 2-methyl-2,4-pentanediamine, 0.5 g. of concentrated sulfuric acid and about 200 ml. of xylene was refluxed in a "water-by-distillation" still for a total of 116 hours at 175°-195° C. after 0.5 mole of water and most of the xylene had been removed. During this time 1.5 moles of water were removed. The reaction mixture was then refluxed for two hours with 20 g. of calcium carbonate, topped, and the residue distilled through a short column at 2 mm. The 2-heptadecyl-4,6,6-trimethyl-3,4,5,6-tetrahydropyrimidine cut was obtained at 184°-200° C/2 mm.

Other species which may be employed in the subject compositions include 2-octadecyl-4,6,6-triethyl-3,4,5,6-tetrahydropyrimidine; 2-dodecyl-6,6-dipropyl-3,4,5,6-tetrahydropyrimidine; 2-carnaubyl-4,6-diamyl-3,4,5,6-tetrahydropyrimidine; 2-heptadecyl-4,5,6,6-tetramethyl-3,4,5,6-tetrahydropyrimidine.

Depending upon the specific pyrimidine, the source of the asphalt and the type of surface to be coated, the amount of the additive to be employed may vary from about 0.1 to 5% by weight of the asphalt. This may be added in unmodified condition or in the form of a solution to the melted asphalt, or may be sprayed or otherwise deposited as a priming coat on the aggregate or other surface as an emulsion or aqueous salt solution or as a solvent.

An unexpected feature distinguishing the subject pyrimidines from other amine-type additives comprises the response which the pyrimidines show to the effect of heat after they have been incorporated in an asphalt. This effect is demonstrated by the examples which follow. It will be noted in Examples 1, 2 and 3 that a heat treatment of one week at 120° C. increased the adhesion characteristics of the pyrimidine employed in many instances. This response to heating is in direct contrast to that noted in Examples 4 and 5, wherein other typical amines were heated after their addition to various asphalts. It has been found that this increase in bonding characteristics is exhibited by asphalt compositions containing the subject pyrimidines when they have been heated for periods longer than about one hour within the temperature range 210-325° C. A convenient means of effecting this heat treatment comprises adding the subject pyrimidines to the asphalt blend and conveying the asphalt to the site where it is to be used in heated tank cars. The examples which follow illustrate the process and products of the present invention and differentiate the results obtained from those which occur when other amines are employed.

#### EXAMPLE 1

The anti-stripping effect of pyrimidines in various asphalts was tested as follows, using a soda rhyolite aggregate:

The  $\frac{1}{4}$ -inch to  $\frac{1}{2}$ -inch crushed, clean aggregate, wet with 2% by weight of water, was mixed with 6% by weight of a medium curing cut-back grade MC-2 asphalt. After curing for one hour at ambient room temperatures, the coated aggregate was covered with distilled water for twenty hours at room temperature, after which

the extent of the surface coating on the aggregate was visually estimated.

The thermal stability of the subject additives was tested under the following conditions. The heating, in the present case, unexpectedly improved the action of the pyrimidines:

The asphalt, containing the pyrimidine, was heated for 168 hours at 120° C. in a closed bottle, conditions which simulate storage in a heated tank or tank car during shipment to a building site, for example. Subsequent to the heat treatment, the above-described coating procedure was carried out. Table I, below, gives the data obtained. The additive employed was 2-heptadecyl-4,6,6-trimethyl-3,4,5,6-tetrahydropyrimidine.

Table I

| Source of Asphalt  | Concentration of Additive, Wt. Per Cent of Asphalt | Per Cent of Aggregate Coated |              |
|--------------------|----------------------------------------------------|------------------------------|--------------|
|                    |                                                    | Not Heat Treated             | Heat Treated |
| San Joaquin Valley | None                                               | 5                            | 5            |
| Do                 | 0.5                                                | 20                           | 85           |
| Do                 | 1.0                                                | 100                          | 98           |
| Texas Gulf         | None                                               | 5                            | 5            |
| Do                 | 0.5                                                | 98                           | 100          |
| Do                 | 1.0                                                | 100                          | 100          |
| Venezuela          | None                                               | 10                           | 10           |
| Do                 | 0.5                                                | 90                           | 100          |
| Do                 | 1.0                                                | 100                          | 100          |
| Mid-Continent      | None                                               | 10                           | 5            |
| Do                 | 0.5                                                | 60                           | 95           |
| Do                 | 1.0                                                | 95                           | 100          |

#### EXAMPLE 2

A set of tests parallel to those described in Example 1 were run but using a granite aggregate. The data obtained are given in Table II, below:

Table II

| Source of Asphalt  | Concentration of Additive, Wt. Per Cent of Asphalt | Per Cent of Aggregate Coated |              |
|--------------------|----------------------------------------------------|------------------------------|--------------|
|                    |                                                    | Not Heat Treated             | Heat Treated |
| San Joaquin Valley | None                                               | 5                            | 100          |
| Do                 | 1.0                                                | 100                          | 100          |
| Texas Gulf         | None                                               | 5                            | 100          |
| Do                 | 0.5                                                | 70                           | 100          |
| Do                 | 1.0                                                | 95                           | 100          |
| Venezuela          | None                                               | 5                            | 10           |
| Do                 | 0.5                                                | 90                           | 95           |
| Do                 | 1.0                                                | 95                           | 100          |
| Mid-Continent      | None                                               | 5                            | 10           |
| Do                 | 1.0                                                | 100                          | 100          |

#### EXAMPLE 3

The tests described in Example 1 were repeated, using a Meramec gravel as the aggregate, with the following results:

Table III

| Source of Asphalt  | Concentration of Additive, Wt. Per Cent of Asphalt | Per cent of Aggregate Coated |              |
|--------------------|----------------------------------------------------|------------------------------|--------------|
|                    |                                                    | Not Heat Treated             | Heat Treated |
| San Joaquin Valley | None                                               | 5                            | 5            |
| Do                 | 0.5                                                | 50                           | 75           |
| Do                 | 1.0                                                | 50                           | 75           |
| Texas Gulf         | None                                               | 10                           | 5            |
| Do                 | 0.5                                                | 80                           | 85           |
| Do                 | 1.0                                                | 80                           | 90           |
| Venezuela          | None                                               | 5                            | 5            |
| Do                 | 0.5                                                | 80                           | 90           |
| Do                 | 1.0                                                | 80                           | 90           |
| Mid-Continent      | None                                               | 5                            | 5            |
| Do                 | 1.0                                                | 80                           | 90           |

5  
EXAMPLE 4

For the purpose of comparison with the anti-stripping stability of the pyrimidine used in Examples 1-3, similar tests were made using a mixture of C<sub>16</sub>-C<sub>18</sub> fatty amines, with the following results; soda rhyolite was the aggregate employed.

Table IV

| Source of Asphalt       | Concentration of Additive, Per Cent by Wt. of Asphalt | Per cent of Aggregate Coated |              |
|-------------------------|-------------------------------------------------------|------------------------------|--------------|
|                         |                                                       | Not Heat Treated             | Heat Treated |
| San Joaquin Valley..... | None                                                  | 5                            | 5            |
| Do.....                 | 0.5                                                   | 95                           | 50           |
| Do.....                 | 1.0                                                   | 95                           | 50           |
| Venezuela.....          | None                                                  | 10                           | 10           |
| Do.....                 | 0.5                                                   | 80                           | 50           |
| Mid-Continent.....      | None                                                  | 10                           | 5            |
| Do.....                 | 0.5                                                   | 65                           | 20           |
| Do.....                 | 1.0                                                   | 90                           | 20           |

## EXAMPLE 5

For comparison with the data obtained in Example 1 with the pyrimidine additive, the tests described therein were repeated, using heptadecylimidazoline as the agent, a soda rhyolite aggregate being coated.

Table V

| Source of Asphalt       | Concentration of Additive, Per Cent by Wt. of Asphalt | Per cent of Aggregate Coated |              |
|-------------------------|-------------------------------------------------------|------------------------------|--------------|
|                         |                                                       | Not Heat Treated             | Heat Treated |
| San Joaquin Valley..... | None                                                  | 5                            | 5            |
| Do.....                 | 0.5                                                   | 80                           | 20           |
| Mid-Continent.....      | None                                                  | 10                           | 5            |
| Do.....                 | 0.5                                                   | 60                           | 10           |
| Do.....                 | 1.0                                                   | 75                           | 30           |

We claim as our invention:

1. A bituminous composition comprising an asphalt and 0.10-5% by weight of a substituted pyrimidine having the general formula



wherein each each R is a substituent of the group consisting of the hydrogen atom and alkyl substituents, at least one of which has at least 10 carbon atoms.

2. A composition according to claim 1 wherein the R radical indicated as R<sub>1</sub> is an alkyl group having more than 10 carbon atoms.

3. A composition according to claim 2 wherein the R radicals indicated as R<sub>2</sub>, R<sub>3</sub> and R<sub>4</sub> are alkyl groups having 1-5 carbon atoms.

4. A composition according to claim 3 wherein the pyrimidine is 2-heptadecyl-4,6,6-trimethyl-3,4,5,6-tetrahydropyrimidine..

5. A bituminous composition comprising an asphalt and 0.1-5% by weight of an alkylated pyrimidine bearing at least one alkyl group having at least 10 carbon atoms.

25 6. A bituminous composition comprising an asphalt and 0.1-5% by weight of 2,4,6,6-tetra-alkyl-3,4,5,6-tetrahydropyrimidine wherein the alkyl radicals in the 2 and 4 positions have 1 to 5 carbon atoms and the alkyl radical in the 6 position has at least 10 carbon atoms.

LLOYD J. MITCHELL.  
HARRY J. SOMMER.

## REFERENCES CITED

35 The following references are of record in the file of this patent:

## UNITED STATES PATENTS

| Number    | Name          | Date          |
|-----------|---------------|---------------|
| 2,191,295 | Dohse et al.  | Feb. 20, 1940 |
| 2,314,111 | Tucker et al. | Mar. 16, 1943 |
| 2,370,286 | Anderson      | Feb. 27, 1945 |

## FOREIGN PATENTS

| Country | Date          |
|---------|---------------|
| France  | July 10, 1939 |